



US006077393A

# United States Patent [19]

Shannon et al.

[11] Patent Number: 6,077,393

[45] Date of Patent: Jun. 20, 2000

[54] **SOFT TISSUE PRODUCTS HAVING HIGH STRENGTH**

[75] Inventors: **Thomas Gerard Shannon**, Neenah; **Nancy Sarsfield Clungeon**, Manawa; **Sheng Hsin Hu**, Appleton, all of Wis.

[73] Assignee: **Kimberly-Clark Worldwide, Inc.**, Neenah, Wis.

[21] Appl. No.: **09/190,317**

[22] Filed: **Nov. 12, 1998**

[51] **Int. Cl.<sup>7</sup>** ..... **D21H 17/45**

[52] **U.S. Cl.** ..... **162/158**; 162/111; 162/179; 162/164.6; 162/168.2; 428/153

[58] **Field of Search** ..... 162/158, 164.6, 162/179, 168.2, 111, 112; 428/152, 153

## [56] References Cited

### U.S. PATENT DOCUMENTS

|           |         |                        |       |         |
|-----------|---------|------------------------|-------|---------|
| 4,940,513 | 7/1990  | Spendel                | ..... | 162/112 |
| 4,959,125 | 9/1990  | Spendel                | ..... | 162/158 |
| 5,354,425 | 10/1994 | Mackey et al.          | ..... | 162/135 |
| 5,607,551 | 3/1997  | Farrington, Jr. et al. | ..... | 162/109 |
| 5,695,607 | 12/1997 | Oriaran et al.         | ..... | 162/112 |

|           |        |                        |       |         |
|-----------|--------|------------------------|-------|---------|
| 5,730,839 | 3/1998 | Wendt et al.           | ..... | 162/111 |
| 5,746,887 | 5/1998 | Wendt et al.           | ..... | 162/109 |
| 5,772,845 | 6/1998 | Farrington, Jr. et al. | ..... | 162/109 |
| 5,882,479 | 3/1999 | Oriaran et al.         | ..... | 162/112 |
| 5,904,810 | 5/1999 | Schroeder et al.       | ..... | 162/111 |

## OTHER PUBLICATIONS

TAPPI Official Test Method T 494 om-88, "Tensile Breaking Properties Of Paper And Paperboard (Using Constant Rate Of Elongation Apparatus)," published by the TAPPI Press, Atlanta, Georgia, revised 1988, pp. 1-5.

*Primary Examiner*—Stanley S. Silverman

*Assistant Examiner*—José A. Fortuna

*Attorney, Agent, or Firm*—Gregory E. Croft

## [57] ABSTRACT

Certain alkylamides and alkylimides, such as hydroxy alkylamides, which ordinarily act as softening agents and substantially reduce the tensile strength of the tissue sheet in accordance with the strength/softness curve, have been found to have a significantly lesser effect on the strength of tissue sheets which have been noncompressively dewatered and dried. As a result, soft uncreped throughdried tissue sheets can be made to have a higher strength:softness ratio by incorporating these chemicals into the furnish.

**13 Claims, 2 Drawing Sheets**



FIG. 1



FIG. 2

**FIG. 3**

## SOFT TISSUE PRODUCTS HAVING HIGH STRENGTH

### BACKGROUND OF THE INVENTION

In the manufacture of tissue products such as facial tissue, bath tissue, paper towels, dinner napkins and the like, it is well known that strength and softness are inversely related. For a given tissue base sheet, increasing the softness of the sheet will generally decrease the tensile strength, particularly when the softness is increased through mechanical or chemical debonding. Creping is a good example of mechanical debonding which substantially weakens the sheet. The addition of debonders to the tissue making furnish is a common example of a chemical means for softening the sheet, but which also results in a weaker sheet. In either case the strength of the tissue sheet must be initially made stronger to counteract the strength degradation of the softening effect. This translates into higher costs for chemical strengthening agents or additional fibers.

Hence there is a need for a means for providing soft tissue sheets which has a less pronounced negative effect on the strength of the resulting sheet.

### SUMMARY OF THE INVENTION

It has now been discovered that certain chemicals, some of which are used in the paper industry as opacifying agents, also act as softener/deboners. Surprisingly, however, it has been found that while these chemicals follow the traditional strength/softness relationship when used in conventional wet pressing processes, when added to the furnish of a tissue making process which uses non-compressively dewatering and drying, the adverse effect on the strength of the tissue sheet is greatly reduced.

Hence in one aspect, the invention resides in a non-compressively dewatered and dried tissue sheet comprising an amount of one or more alkylamide and/or alkylimide softening agents having at least one of the following structures:



wherein R=any saturated or unsaturated fatty acid group having a chain length of 6 to 22 carbon atoms;

n=0,1;  
x=to 6;  
y=1to 6;  
Z=H, OH; and

A=any anion of a strong or weak acid.

In another aspect, the invention resides in a method of making a soft and strong tissue sheet comprising:

(a) adding one or more alkylamide or alkylimide softening agents to an aqueous suspension of papermaking fibers and maintaining the resulting aqueous mixture of fibers and alkylamides at a temperature of from about 20° C. to about 70° C. for at least 10 minutes, said softening agent(s) having one or more of the following structures:

(1)



(2)



(3)



wherein R=any saturated or unsaturated fatty acid group having a chain length of 6 to 22 carbon atoms;

n=0,1;

x=1 to 6;

y=1 to 6;

Z=H, OH; and

A=any anion of a strong or weak acid;

(b) depositing the aqueous suspension of papermaking fibers onto a forming fabric to form a tissue web;

(c) non-compressively dewatering the web; and

(d) non-compressively drying the web to form a soft tissue sheet.

Suitable commercially available alkylamides are sold under the trade name Reactopaque® 100, 102 and 115 by Sequa Chemical Company, Chester, S.C., which are sold as aqueous solutions. These three materials are believed to be blends of the alkylamides set forth in structural formulas (1) and (2) above. Reactopaque® 102 is about 20 weight percent solids, Reactopaque® 100 is about 10 weight percent solids, and Reactopaque® 115 is about 15 weight percent solids.

The amount of the alkylamide or alkylimide softening agent, on a solids basis, used to attain improved strength and softness can be from about 0.5 to about 30 pounds per metric ton of fiber, more specifically from about 2 to about 20 pounds per metric ton of fiber, and most specifically from 6 to about 15 pounds per metric ton of fiber. Preferred amounts are greater than the amounts recommended for purposes of improving opacity in writing papers and newsprint, which are the primary market for these materials.

In mixing the alkylamide and/or the alkylimide with the aqueous suspension of papermaking fibers, it is desirable to maintain the mixture in a heated condition for a period of time before forming the tissue web. The temperature of the aqueous fiber suspension/alkylamide mixture can be from about 20° C. to about 90° C., more specifically from about 30° C. to about 80° C., and still more specifically from about 40° C. to about 70° C. The length of time that the mixture is maintained at the elevated temperature can be about 5 minutes or longer, more specifically from about 5 minutes to about 40 minutes, and still more specifically from about 5 minutes to about 20 minutes.

The alkylamides and/or alkylimide softening agents can be mixed with the entire furnish used to make the tissue or they can be added to select portions of the furnish, such as the furnish of one or more layers of a layered tissue. Alternatively, the amounts of the softening agents can be the same or different in each of the furnish layers.

The GMT (Geometric Mean Tensile strength expressed as grams-force per 3 inches of sample width) of the tissue sheets of this invention can be about 600 or greater, more specifically about 700 or greater, still more specifically about 800 or greater, still more specifically about 1000 or greater, and still more specifically from about 700 to about 1300. GMT is computed from the peak load values of the

MD (machine direction) and CD (cross-machine direction) tensile curves, which are obtained under laboratory conditions of 23.0+/-1.0 degrees Celcius and 50.0+/-2.0 percent relative humidity and only after the sheet has equilibrated to the testing conditions for a period of not less than four hours. Testing is done on a constant rate of elongation tensile testing machine. Specimen width is 3 inches. Jaw span (the distance between the jaws, sometimes referred to as gauge length) is 2.0 inches (50.8 mm.) Crosshead speed is 10 inches per minute (254 mm/min.) A load cell/full scale load is chosen so that the majority of peak load results fall between 20 and 80 percent of the full scale load. In particular the results described here were produced on an Instron 1122 tensile frame connected to a Sintech data acquisition and control system utilizing IMAP software running on a '486 Class' personal computer. This data system records at least 20 load and elongation points per second.

The MD Slope of the tissue sheets of this invention can be about 10 or less, more specifically about 9 or less, and still more specifically from about 4 to about 8. The MD Slope is the two parameter least squares line regression coefficient (sometimes referred to as slope) obtained from the tensile load/elongation curve for all points falling between a load of 70 grams and 157 grams during the ascending part of the curve. The regression coefficient is multiplied by the jaw span and divided by the specimen width to normalize the result, resulting in the final MD Slope value. The MD Slope values may be obtained from the MD tensile curves utilized for the GMT calculation; MD Slope utilizes an identical 3 inch specimen width and two inch jaw span. The units for MD Slope are kilograms per 3 inches (7.62 centimeters), but for convenience, the MD Slope values are hereinafter referred to without units.

The MD Stiffness Factor of the products of this invention can be about 100 or less, more specifically about 80 or less, and still more specifically from about 40 to about 80. The MD Stiffness Factor is calculated by multiplying the MD Slope by the square root of the Caliper (measured as described below). The units of the MD Stiffness Factor are (kilograms per 3 inches) microns<sup>0.5</sup>, but for simplicity the values of the MD Stiffness Factor are hereinafter referred to without units.

For purposes of calculating the MD Stiffness Factor, the Caliper is the thickness of a single sheet, expressed in microns. It is measured under laboratory conditions of 23.0+/-1.0 degrees Celcius and 50.0+/-2.0 percent relative humidity and only after the sheet has equilibrated to the testing conditions for a period of not less than four hours. The micrometer used for carrying out this measurement is an Emveco model 200-A with flat ground, circular pressure foot and anvil and with factory modifications to meet the following specifications: a round pressure foot diameter of 56.42 millimeters (equating to an area of 2500 square millimeters; pressure foot loading of 2.00 kilopascals; 0 to 7.6 mm test capacity; readout resolution of 0.001 millimeters; repeatability of 0.001 millimeters;

linearity of +/-0.25 percent; dwell time of 3.0+/-1.0 seconds; lowering rate of 0.8 millimeters +/-0.1 per second; and pressure foot and anvil to be parallel within 0.001 mm.

The MD Stiffness Factor: GMT ratio, expressed in kg-microns<sup>0.5</sup>/gm, for tissue sheets in accordance with this invention can be about 0.077 or less, more specifically about 0.060 or less, more specifically about 0.050 or less, and more specifically from about 0.030 to about 0.070, and still more specifically from about 0.050 to about 0.070.

#### BRIEF DESCRIPTION OF THE DRAWINGS

FIG. 1 is a plot of softness versus strength for non-compressively dewatered and dried tissue sheets comparing the strength loss effect of conventional (imidazoline

quaternary) softening agents with that of certain alkylamide softening agents in accordance with this invention. As shown, the imidazoline quaternaries follow the typical strength/softness curve, while the alkylamides of this invention are off of the curve and represent increased strength for a given level of softness.

FIG. 2 is a bar chart comparing the percent tensile loss for pressed and unpressed handsheets as a function of the add-on amount of certain alkylamide softening agents in accordance with this invention. As shown, at the same wet end add-on amounts, the non-compressively dewatered sheets had substantially less strength loss than the wet-pressed sheets.

FIG. 3 is a plot of the MD Stiffness Factor versus GMT for several tissue base sheets (not converted into final product form), illustrating how steeply the curve rises for the oleyl imidazoline quaternaries as compared to the relatively flat curves for tissue sheets made in accordance with the alkylamides of this invention (R-115 and R-150). The flatter curves illustrate how greatly increased strength can be achieved with a relatively small increase in stiffness (lower loss of softness). Also noteworthy in FIG. 3 is the impact of adding a relatively small amount of alkylamide softening agent in conjunction with an oleyl imidazoline softening agent. An almost 50 percent reduction in stiffness factor is seen with addition of 2 pounds of the alkylamide per metric ton of fiber.

#### EXAMPLES

##### Example 1

(Control).

A one-ply, non-layered, uncreped throughdried tissue basesheet was made generally in accordance with U.S. Pat. No. 5,607,551 issued March 4, 1997 to Farrington et al. entitled "Soft Tissue", which is herein incorporated by reference. More specifically, 60 pounds (oven dry basis) of eucalyptus hardwood kraft fiber and 40 pounds (oven dry basis) of northern softwood kraft fiber were dispersed in a pulper for 30 minutes at a consistency of 3 percent. The thick stock slurry was then passed to a machine chest and diluted to a consistency of 1 percent. To the machine chest was added 182 grams (8.8 pounds per metric ton of dry fiber) of a commercially available dry strength resin, Parez 631-NC. The dry strength resin was added as a 6 percent aqueous solution. The stock was further diluted to approximately 0.1 percent consistency prior to forming. The formed web was non-compressively dewatered and rush transferred to a transfer fabric traveling at a speed about 25 percent slower than the forming fabric. The web was then transferred to a throughdrying fabric, dried and calendered. The total basis weight of the resulting sheet was 16 pounds per 2880 ft<sup>2</sup>.

##### Example 2

(Invention).

A single-ply, non-layered uncreped throughdried tissue basesheet was made as described in Example 1, except the fibers were initially dispersed in a pulper for 5 minutes at a consistency of 3 percent. The temperature of the water in the pulper was raised to 120° F. (49° C.) prior to addition of the pulp. 275 grams of a 15 percent aqueous solution (41.3 grams dry basis, 2 pounds per metric ton of dry fiber) of a commercially available alkylamide softening agent (Reactopaque® 115 manufactured by Sequa Chemical Company) was added to the pulper and the pulp was allowed to disperse for 25 additional minutes.

## 5

## Example 3

(Invention).

Same as Example 2, except that 825 grams of Reactopaque 115 (123.9 grams dry basis, 6 pounds per metric ton of dry fiber) was added to the pulper.

## Example 4

(Invention).

Same as Example 2, except that 2063 grams of Reactopaque 115 (309.5 grams dry basis, 15 pounds per metric ton of dry fiber) was added to the pulper.

## Example 5

(Conventional softening agent).

Same as Example 1, except that after the addition of the Perez dry strength resin to the machine chest, 41.3 grams (2 pounds per metric ton dry fiber) of a commercially available quaternary ammonium oleyl imidazoline softening agent (C-6001, Witco Corporation) was added. The softening agent was added as a 4 percent aqueous solution.

## Example 6

(Conventional softening agent):

Same as Example 5, except that 82.6 grams of the oleyl imidazoline softening agent (4 pounds per metric ton of fiber) was added to the machine chest as a 4 percent aqueous solution.

## Example 7

(Conventional softening agent).

Same as Example 5, except that 125 grams of the oleyl imidazoline softening agent (6 pounds per metric ton of dry fiber) was added to the machine chest as a 4 percent aqueous solution.

The tissues produced by Examples 1-7 were tested for softness by a trained sensory panel and for geometric mean tensile (GMT) strength, which is expressed as grams-force per 3 inches of sample width. The add-on level (Level) of the softening agent is expressed as pounds per metric ton of fiber on a dry basis. The results are set forth in TABLE 1 below:

## 6

The results of TABLE 1 illustrate that the alkylamide softening agents of this invention can attain equivalent softness at greater strength than the oleyl imidazoline softening agents.

## Example 8

(Control—Creped/Wet-pressed).

A two-ply, wet-pressed bath tissue having a basis weight of 19 pounds per 2880 ft<sup>2</sup>. was made in a conventional manner. More specifically, 60 pounds (oven dry basis) of eucalyptus hardwood kraft fiber and 40 pounds (oven dry basis) of northern softwood kraft fiber were dispersed in a pulper for 30 minutes at a consistency of 3 percent. The thick stock slurry was then passed to a machine chest and diluted to a consistency of 1 percent. To the machine chest was added 10.3 grams (0.5 pounds per metric ton of dry fiber) of a commercially available wet strength resin, Perez 631-NC, and 41.3 grams (2 pounds per metric ton of dry fiber) of a commercially available dry strength resin, Redibond 2005, and 49.6 grams (2.4 pounds per metric ton of dry fiber) of a commercially available imidazoline softening agent (C-6027 from Witco Corporation). The stock was further diluted to about 0.1 % consistency prior to forming, dewatering, drying and creping of the tissue web, which was plied together with a like web and calendered to form the final two-ply tissue product.

## Example 9

(Hydroxy alkylamide/wet-pressed).

Same as Example 8, except that 163.2 grams dry basis (8 pounds per metric ton of dry fiber) of a commercially available alkylamide softening agent, Reactopaque 102, was added to the pulper.

## Example 10

(Uncreped Throughdried Control).

A one-ply, non-layered, uncreped throughdried tissue basesheet was made generally in accordance with U.S. Pat. No. 5,607,551 issued Mar. 4, 1997 to Farrington et al. entitled "Soft Tissue", which is herein incorporated by reference. More specifically, 50 pounds (oven dry basis) of eucalyptus hardwood kraft fiber and 50 pounds (oven dry

TABLE 1

| Example                      | Softening Agent                           | Level | GMT     | Panel Softness | Strength loss vs. Control |
|------------------------------|-------------------------------------------|-------|---------|----------------|---------------------------|
| 1<br>(Control)               | none                                      | 0     | 1641    | —              | —                         |
| 2<br>(Invention)             | hydroxy alkylamide<br>(Reactopaque ® 115) | 2     | 1268    | —              | 22.7                      |
| 3<br>(Invention)             | hydroxy alkylamide<br>(Reactopaque ® 115) | 6     | 1005    | —              | 38.9                      |
| 4<br>(Invention)             | hydroxy alkylamide<br>(Reactopaque ® 115) | 15    | 851/740 | 9.4            | 48.4                      |
| 5<br>(Conventional debonder) | oleyl imidazoline (C-6001)                | 2     | 716/600 | 9.1            | 56.6                      |
| 6<br>(Conventional debonder) | oleyl imidazoline (C-6001)                | 4     | 660/540 | 10.0           | 60.0                      |
| 7<br>(Conventional debonder) | oleyl imidazoline (C-6001)                | 6     | 618/490 | 10.8           | 62.5                      |

Note: The first GMT value listed is for the base sheet, while the second value is for the converted bath tissue product, which has been calendered.

basis) of northern softwood kraft fiber were dispersed in a pulper for 30 minutes at a consistency of 3 percent. The thick stock slurry was then passed to a machine chest and diluted to a consistency of 1 percent. The stock was further diluted to approximately 0.1 percent consistency prior to forming. The formed web was non-compressively dewatered and rush transferred to a transfer fabric traveling at a speed about 25 percent slower than the forming fabric. The web was then

basesheets were made as described above in Example 10, but using different amounts of softening agents. The GMT, MD Max Slope, and MD Stiffness Factor were measured for each sample. The results are summarized in TABLE 3 below.

5 As above, the add-on level (Level) of the softening agent is expressed as pounds per metric ton of fiber on a dry basis. All of the samples containing additives designated as "R-115" or "R-150" are in accordance with this invention.

TABLE 3

| Example | Softening Agent                  | Level | GMT  | MD Slope | MD Stiffness Factor | MD Stiffness Factor: GMT Ratio (Kg-microns <sup>0.5</sup> )/gm |
|---------|----------------------------------|-------|------|----------|---------------------|----------------------------------------------------------------|
| 12      | none                             | 0     | 1641 | 16.31    | 186                 | 0.113                                                          |
| 13      | C-6001                           | 2     | 716  | 8.67     | 99                  | 0.138                                                          |
| 14      | C-6001                           | 4     | 660  | 6.16     | 70                  | 0.106                                                          |
| 15      | C-6001                           | 6     | 618  | 4.32     | 49                  | 0.079                                                          |
| 16      | R-115                            | 2     | 1268 | 7.45     | 85                  | 0.067                                                          |
| 17      | R-115                            | 6     | 1005 | 7.32     | 83                  | 0.082                                                          |
| 18      | R-115                            | 15    | 851  | 5.78     | 66                  | 0.077                                                          |
| 19      | R-150                            | 2     | 1224 | 6.54     | 75                  | 0.061                                                          |
| 20      | R-150                            | 4     | 995  | 4.93     | 56                  | 0.056                                                          |
| 21      | R-150                            | 6     | 775  | 5.16     | 59                  | 0.076                                                          |
| 22      | 2 pounds R-115 + 4 pounds C-6001 | 6     | 683  | 3.80     | 43                  | 0.063                                                          |

transferred to a throughdrying fabric and dried. The total basis weight of the resulting sheet was 16 pounds per 2880 ft<sup>2</sup>.

#### Example 11

(Invention).

A single-ply, non-layered uncreped through dried tissue basesheet was made as described in Example 10 with the exception that 165.2 grams dry basis (8 pounds per metric ton of dry fiber) of a commercially available softening agent, Reactopaque 102, was added to the pulper.

The tissue products of Examples 8-11 were tested for GMT strength and the results are set forth in TABLE 2. As above, the add-on level (Level) of the softening agent is expressed as pounds per metric ton of fiber on a dry basis.

TABLE 2

| Example | Method       | Alkylamide Softening Agent | Level | GMT  | Strength Loss |
|---------|--------------|----------------------------|-------|------|---------------|
| 8       | wet-press    | none                       | 0     | 1391 | —             |
| 9       | wet-press    | yes                        | 8     | 613  | 55.9          |
| 10      | throughdried | none                       | 0     | 950  | —             |
| 11      | throughdried | yes                        | 8     | 840  | 11.6          |

The results of TABLE 2 illustrate that in a conventional wet-pressing process the use of alkylamide softening agents causes significant debonding and weakening of the sheet with a 55.9 percent loss in tensile strength. However, in a process not involving compressive dewatering, the use of alkylamide softening agents in accordance with this invention demonstrate significantly less debonding and weakening of the sheet. In the example above only a 11.6 percent tensile loss was observed for the same level of addition.

#### Examples 12-22.

To further illustrate the unique combination of softness and strength attained using the alkylamide softening agents in accordance with this invention, throughdried tissue

30 These results illustrate the unique combination of strength and softness (as measured by the MD Slope and the MD Stiffness Factor) achieved using tissues containing the alkylamides of this invention.

35 It will be appreciated that the foregoing examples, given for purposes of illustration, shall not be construed as limiting the scope of this invention, which is defined by the following claims and all equivalents thereto.

We claim:

1. A non-compressively dewatered and dried tissue sheet comprising an amount of one or more alkylamide and/or alkylimide softening agents having at least one of the following structure(s):



45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335

2. The tissue of claim 1 wherein the amount of the softening agent, on a solids basis, is from about 0.5 to about 20 pounds per metric ton of dry fiber.

3. The tissue of claim 1 wherein the amount of the softening agent, on a solids basis, is from about 2 to about 20 pounds per metric ton of dry fiber. 5

4. The tissue of claim 1 wherein the amount of the softening agent, on a solids basis, is from 6 to about 15 pounds per metric ton of dry fiber.

5. The tissue of claim 1 wherein  $Z=OH$ .

6. A non-compressively dewatered and dried tissue sheet comprising an amount of an alkylamide softening agent having the following structure: 10



wherein R=any saturated or unsaturated fatty acid group having a chain length of 6 to 22 carbon atoms; 15

$n=0,1$ ;

$x=1$  to 6;

$y=1$  to 6; and

$Z=H$  or  $OH$ ,

wherein the softening agent imparts a substantially lower percent tensile loss to non-compressibly dried handsheets than to comparable wet-pressed hand sheets at an add-on level of from 5 to 20 pounds per metric ton of dry fiber. 20

7. The tissue of claim 6 wherein the alkylamide has the following structure:



8. A non-compressively dewatered and dried tissue sheet comprising an amount of an alkylamide softening agent having the following structure: 35



wherein R=any saturated or unsaturated fatty acid group having a chain length of 6 to 22 carbon atoms; 45

$n=0,1$ ;

$x=1$  to 6;

$y=1$  to 6;

$Z=H$  or  $OH$ ; and

$A=$ any anion of a strong or weak acid, wherein the softening agent imparts a substantially lower percent tensile loss to non-compressibly dried handsheets than to comparable wet-pressed handsheets at an add-on level of from 5 to 20 pounds per metric ton of dry fiber. 50

9. The tissue of claim 8 wherein the alkylamide has the following structure:



10. The tissue of claim 9 further comprising an alkylamide softening agent having the following structure: 65



wherein R=a saturated or unsaturated fatty acid alkyl group having a chain length of 6 to 22 carbon atoms.

11. A non-compressively dewatered and dried tissue sheet comprising an amount of an alkylamide softening agent having the following structure: 10



wherein R=any saturated or unsaturated fatty acid group having a chain length of 6 to 22 carbon atoms;

$n=0,1$ ;

$x=1$  to 6;

$y=1$  to 6;

$Z=H$  or  $OH$ ; and

$A=$ any anion of a strong or weak acid,

wherein the softening agent imparts a substantially lower percent tensile loss to non-compressibly dried handsheets than to comparable wet-pressed handsheets at an add-on level of from 5 to 20 pounds per metric ton of dry fiber. 25

12. The tissue of claim 11 wherein the alkylamide softening agent has the following structure:



13. A method of making a soft and strong tissue sheet comprising:

(a) adding an amount of one or more softening agents to an aqueous suspension of papermaking fibers and maintaining the resulting aqueous mixture of fibers and softening agent(s) at a temperature of from about 40° C. to about 70° C. for at least 5 minutes, said

softening agent(s) having one or more of the following structures:



(1)



(2)



(3)

wherein R=any saturated or unsaturated fatty acid group having a chain length of 6 to 22 carbon atoms;

$x=1$  to 6;

$y=1$  to 6;

Z=H, OH; and

A=an anion of any strong or weak acid;

- (b) depositing the aqueous suspension of papermaking fibers onto a forming fabric to form a tissue web;
- (c) non-compressively dewatering the web; and
- (d) non-compressively drying the web to form a soft tissue sheet,

wherein the softening agent imparts a substantially lower percent tensile loss to non-compressibly dried handsheets than to comparable wet-pressed handsheets at an add-on level of from 5 to 20 pounds per metric ton of dry fiber.

\* \* \* \* \*